

Jan. 6, 1970

J. F. CLARKE

3,487,521

## ALLOY FOIL

Filed Oct. 4, 1967



FIG. 2

John F. Clarke,  
Inventor.  
Koenig, Senniger, Powers and Learith,  
Attorneys.

## 1

3,487,521  
ALLOY FOIL

John F. Clarke, Attleboro, Mass., assignor to Texas Instruments Incorporated, Dallas, Tex., a corporation of Delaware

Filed Oct. 4, 1967, Ser. No. 672,809  
Int. Cl. C22c 33/02, 39/02, 1/05

U.S. Cl. 29—182.5

1 Claim

### ABSTRACT OF THE DISCLOSURE

A flexible metal supporting strip is coated with a slurry composed of powders of different alloyable metals, a high-molecular-weight binder and a carrier liquid. The alloys to be formed are often brittle. After drying, the slurry is compressed sufficiently on the strip to green-bond the particles of the alloyable powders to one another but without embrittling alloying. The dried slurry is then freed from the supporting strip by peeling it therefrom. It is then sintered by heating to a temperature high enough to improve the green-bonds, but not high enough to effect alloying of the metal particles. It is then rolled for compaction to final gauge and again sintered at a temperature high enough to homogenize by diffusion all of the constituent particles to form a free homogenous alloy sinter in nonporous foil form, characterized by the absence of directional grain.

The invention relates to the product hereinafter described, the scope of the invention being indicated in the appended claims.

Heretofore it has not been possible to easily produce a dense, thin, substantially pore-free, rolled alloy foil which is without directional grain and of uniform thickness. More particularly it has not been possible to obtain a rolled alloy foil in which the alloy is brittle and without such directional grain. This is for the reason that rolling has been resorted to on the pre-alloyed composition which if brittle resulted in cracking due to the rolling. My new alloy foil is of the variety which may be brittle when made of certain alloyable components. Brittleness in the alloy is not always a disadvantage where the foil is being used, for example, for brazing or as conductive material on a circuit board. However, the foil whether brittle or not should preferably be without a directional grain. Directional grain would be undesirable, for example, in circuit board applications, because the etching that is required in such cases will not be uniform. Thus the property of being without directional grain is useful.

My new foil is made by an improved apparatus and method for manufacturing improved thin sheets or foils of alloys from powders of the constituent metals, where-in uniformity of thickness and alloy composition is obtained throughout the foil. The strip from which the foil is made remains ductile during rolling to avoid cracking. It is not rolled after homogenization to form the desired alloy thereby avoiding the undesirable directionally grained property. Thus homogenization to effect alloying of metal components which may cause brittleness is delayed until certain rolling steps have been completed.

## 2

In the following description foil refers to thin sheet-metal alloy, the thickness being a few thousandths of an inch, usually about 0.001" to 0.008" or so. Powder means a finely divided substance. The average particle size is less than 50 microns with substantially no particles exceeding 100 microns in size. The exact size of the particles depends on the hardness of the metals involved, and the shape of the powder particles. The term slurry means a liquid medium of substantial viscosity containing metal particles suspended in a binder. The term binder means long-chain, high-molecular-weight organic compounds or the like characterized in that their constituents when comminuted are stringy and when mixed with a liquid such as water act according to the invention to hold or bind the metal particles in suspension and to produce adequate viscosity in the slurry for adherence to a smooth surface. Thus the slurry will adhere evenly to metal surfaces contacted by it. Examples, but without limitation, of suitable binders are methyl cellulose, nonionic cellulose ether, polyethylene oxide, polyvinyl pyrrolidone et cetera. The intended use of the foil will determine the particular gauge to which it is manufactured. The drawings are illustrative and not to scale because of the small dimensions involved.

Briefly, the process for manufacturing foil according to the invention comprises coating a flexible preferably metal carrier strip with a slurry containing particles or powders of several different metals suspended in a binder, solidifying the slurry by heating to dry it, compacting and sintering it at a relatively low temperature to green-bond particles, and then compacting and sintering it a second time at a relatively high temperature to alloy the metals. The slurry includes a mixture of a long-chain, high-molecular-weight organic compound acting as a binder, a carrier such as water, and powders of the constituent metals to make the desired alloy. When foil of an alloy is being manufactured, the powders of each of the various elemental metals of the alloy are supplied to the slurry in the proportion desired in the resulting alloy. The particles by mixing are evenly suspended by the binder. The amount of the binder used controls the viscosity of the slurry so that when applied to a metal surface it will cling thereto. For example, its viscosity may be from 1000 to 4000 cps. The percentage of solids therein may be 50% to 75%. The object of this is that when evenly applied, the slurry will remain substantially even in any position of the metal surface. In some but not all cases a conventional wetting agent such as an aerosol may be used to advantage in the slurry.

In the accompanying drawings, in which one of various possible embodiments of the invention is illustrated:

FIG. 1 is a diagrammatic view, parts being broken away, illustrating apparatus and steps for manufacturing metal strip or foil in accordance with the invention; and

FIG. 2 is a view illustrating diagrammatically modifications of certain materials which occur as they pass through the process.

Corresponding reference characters indicate corresponding parts throughout the several views of the drawings.

Referring now to FIG. 1 of the drawings, a flexible metal carrier strip 1 is unwound from a reel 3 and fed to a roller coater generally designated 5 for receiving a

coating of the slurry. Ultimately the carrier strip 1 is rewound on a reel 6. The carrier strip is preferably composed of a hard metal, such as cold-rolled stainless steel, but if desired may be made of other appropriate material. It may be in the range of from .005" to .050" or so.

The roller coater 5 comprises a reservoir 7 which receives slurry 9 after it has been thoroughly mixed. The coater has two passages 11 and 13 through which the slurry is delivered to an upper trough 15 and a lower trough 17, respectively. As carrier strip 1 moves through the coater 5 in the direction indicated by the arrows in FIG. 1, it passes between spaced upper and lower rollers 19 and 21 which are rotating in the direction indicated by the arrows. Roller 19 is at one side of trough 15 and is spaced from a metering roller 23 at the other side of the trough. The gap between rollers 19 and 23 determines the amount of slurry carried by the roller 19 to the top side of carrier 1. Similarly, roller 21 is above trough 17 and the distance it is spaced from metering roller 25 beneath the trough determines the amount of slurry carried by roller 21 to the underside of the carrier 1. With rollers 19, 21, 23 and 25 rotating in the directions indicated by the arrows, the upper and lower surfaces 1A, 1B (FIG. 2) of the carrier become uniformly coated with layers of slurry 9 from the troughs 15 and 17. The wet slurry coatings applied to carrier 1 are indicated at 29 and 31 in FIG. 2. By changing the spacing between the pairs of rollers at each trough, the amount of slurry metered to the carrier and thus the thickness of the coatings 29 and 31 may be varied. Preferably the coatings are substantially the same thickness but may be different. The coatings are held on the carrier at this time by the binder which adheres to the surfaces 1A and 1B (FIG. 2) of the carrier. Coating thickness may be .010", for example, when wet.

Next the coatings 29, 31 are dried on the carrier. The dried coatings are designated 30, 32. The means illustrated in the drawings for drying the wet coatings 29 and 31 comprise resistance heating of the strip 1 by connecting a source of electric current 33 to the strip 1 through conductors 35, 37, including brushes, as indicated at 8 and 10. The electrical resistance strip 1 results in heat being conducted to the wet coatings 29 and 31 which as they move forward reach the dry condition 30 and 32. While the thickness of coatings 29 and 31 may vary, a dried thickness at 30 and 32 of about 0.005" or 0.006" for each coating has been found satisfactory for producing a final foil thickness of about .0015" to .002".

Strip 1 with the dried coatings 30 and 32 thereon is then passed between rolls 39, 41 of a conventional roller mill. Rolls 39, 41 compact the coatings 30 and 32, thereby reducing their thickness and increasing their density in the aggregate, as indicated at 34 and 36. Preferably these rolls 39, 41 effect a reduction in the dry coating thickness in the range of from 10% to 50% or more. Thus a thickness of about .0025" to .003" may be obtained from an original thickness of about 0.006", which is satisfactory. The dry coatings 30 and 32 are compacted in the rolling mill an amount sufficient to effect sufficient green bonding in the solid phase between adjacent particles of metal in the coating, thereby providing a sufficiently cohesive metallic structure to be handled in the remainder of the process. However, the particles do not green-bond to the strip 1 because of the particle size, shape and hardness. It will be understood that bonding of the particles to the strip is inhibited by the following characteristics: softness of the particles in relation to the strip, certain particle shapes such as flat or acicular, and small particle size. It will be understood that the pressure required for the requisite reduction of the dried slurry is preferably not such as to reduce the thickness of the backing strip 1.

The coatings 30 and 32, when dried and compacted by reduction as at 34 and 36, are peeled from strip 1. The carrier strip 1 is then wound on reel 6 and, since the coating has not bonded to the carrier strip during compaction by the rolling mill, the carrier strip can be reused with little or no cleaning or other work being performed on it. Stripping of the compacted dried coatings 34 and 36 from the carrier strip 1 is facilitated by guide rollers 4 and a naturally occurring curling phenomena sometimes called "alligatoring." This is the tendency of two sheets being rolled to curl away from one another at the roll exit. Thus the dry coating 34 tends to curl up as viewed in FIG. 1 while the dry coating 36 tends to curl down, thus facilitating drawing away of the coatings from the carrier strip.

Next coating 34 is sintered in a furnace 43 and the coating layer 36 is sintered in a furnace designated 45, being guided by rollers 4. Furnaces 43 and 45 may be conventional heating furnaces for sintering and may be provided with inert protective or reducing atmospheres such as argon, hydrogen or the like, depending upon the nature of the metal constituting the starting powdered metal. Coatings 34 and 36 are sintered at a temperature which is sufficient to remove by vaporization most, if not all, dried binder in the coating, and by diffusion and grain growth effecting improvement of the solid-phase green bonds between metal particles of at least one of the metal powder elements in the coating. However, the sintering temperature is low enough to prevent any substantial homogenization or alloying between particles of different elements in the coatings. Any substantial diffusion of unlike particles of metal in the layers to homogenize and alloy such particles at this time is avoided, since it would cause embrittlement of the coatings 34 and 36 and make it difficult further to process. The coatings at this stage are designated 38 and 40 in FIG. 2.

Next the coating 38, which at this time is not brittle, is compacted to the desired final gauge of the strip or foil by passing the coating between two squeeze rolls 47 and 49 of a conventional rolling mill. In a similar manner the coating 40 is compacted to final gauge by a pair of squeeze rolls 51 and 53. The density of the coatings is somewhat increased as a result of this second compaction. Another purpose is smoothing and final sizing. In this case reduction may be 5% to 40% or so. The compacted coatings are designated 42 and 44. The coatings may be rolled at this time without difficulty since they are still ductile.

After the coatings 42 and 44 are rolled to final gauge, they are heated in furnaces 55 and 57 at a temperature higher than the temperature in the furnaces 43 and 45. The temperature in furnaces 55 and 57 is sufficient to homogenize all of the constituent particles to form the desired alloy. This occurs by substantially complete diffusion between all like and unlike particles of constituent metals in the coatings. The finished strips or foils of metal or metal alloys are designated 46, 48 and they may be wound into coils as shown at 59 and 61. The resulting strips 46, 48 are very dense and substantially pore-free. The final alloying may cause embrittlement of the foil, but this is not detrimental since manufacture of the foil is complete.

The following is a particular example of how the process of the invention has been performed to make a brazing alloy which is brittle.

A slurry for a nickel-based brazing alloy was prepared containing by weight 4.5% silicon powder, 3.5% boron powder and 92% nickel powder. These ratios are equivalent to those in the known AMS 4778 brazing alloy. The element metal powders were mixed with a polyethylene oxide binder and water as a solvent. The nickel used was a carbonyl nickel (INCO type 255 or the equivalent) which, being fine, i.e., 2 to 14 microns in average particle size, is easily sintered at low temperatures over a short period

of time. This also favors later stripping away from carrier 1. The slurry was thoroughly mixed and placed in reservoir 7 of reverse roller coating apparatus 5. Thus a thin coating of the slurry (about .010") was applied to each surface of a hard, cold-rolled stainless steel carrier.

The coatings were dried on the carrier by resistance heating of the carrier (as shown at 30, 32). The dried thickness was about .005". The dried coating was then rolled down to about .0025" to compact the coatings (as illustrated at 34, 36 in FIG. 2 of the drawings). This effected initial green bonding between the particles themselves. Due to the small average size of the metal particles, there was no bonding between the metal particles and the carrier. Compaction of the coatings was accomplished without the rolls 39, 41 touching strip 1 and without reduction in its thickness.

The green-bonded compacted coatings were peeled off the carrier strip as they left the rolling mill and then passed through the first sintering furnaces such as shown at 43 and 45. The green bonded compacts were sintered in furnaces 43, 45 at a temperature of about 1400° F. for about 30 seconds to one minute, which was sufficiently high to cause densification of the foil or coating layer and substantially increase in the nickel-to-nickel bonds in the coatings. Some shrinking occurred to .002". This is illustrated in FIG. 2 of the drawings, where the portion of the coatings designated 38, 40 diagrammatically illustrates nickel particles bonded together as a matrix with the Si and B particles held therein. Sintering in the first furnaces 43 and 45 removed a major part of the binder, leaving a dense layer. However, the temperature in furnaces 43 and 45 was beneath the temperature at which sufficient diffusion could take place between particles of the three powders to form any brittle alloy. Diffusion between these unlike particles at this time would cause embrittlement of the foil and make it difficult to effect final processing. The partially sintered strips were then rolled to finished gauge of about .0015" by the rolls 47, 49, 51 and 53. These rolls perform what is sometimes called a kiss pass, meaning that it smooths and finally sizes the product to foil dimensions. However, the kiss pass may reduce thickness as much as 40% or so. Finished foil thicknesses of from about 0.001" to 0.008" have been made successfully. Brazing foils are normally used at thicknesses in that range. Next the product was resintered in furnaces such as 55 and 57 for 30 seconds to one minute at a higher temperature of about 1600° F. to homogenize and alloy by diffusion of the three different metals in the coating and by grain growth to bring about alloying. The times consumed in the furnaces are variable, depending upon temperature and the metals that are being sintered. Thirty seconds to a minute is generally satisfactory.

Self-sintering of the type 255 INCO nickel powders referred to above occurs at approximately 1200° F. On the other hand, nickel-silicon-boron homogenization taken place rapidly above 1500° F. Therefore, by selecting said type 255 nickel powder (or the equivalent) I have been able to produce a strong metal foil by first sintering the coating or foil at about 1400° F. (in the furnaces designated 43 and 45) and then resintering the foil (after it is rolled to finished gauge) at about 1600-1700° F. to produce a homogeneous nickel-silicon-boron alloy which melts completely during brazing at about 1950° F. The finished foil is very dense and substantially pore-free.

By delaying homogenization of the unlike metal particles forming the alloy until after the alloy has been rolled to its finished thickness, brittleness does not occur until after final gauge is obtained. Thus the coating or strip being produced is easily worked to the desired gauge by conventional equipment, whereas subsequent to homogenization of the alloy the strip may be too brittle to process except by special equipment or processes. The strip or foil manufactured by my process is almost 100% metal, the binder and solvent having been vaporized and

removed by heating during drying the the coatings and/or by heating in the sintering furnaces.

Another brazing alloy that may be made according to the invention is one constituted by nickel, silicon and chromium particles, the chromium being substituted for the boron in the above-described process. The weight ratio of nickel to silicon to chromium is 71-10-19. Temperatures used in the process in this case are like those above given, except that homogenization takes place at about 1700° F.-1800° F., the temperature employed for brazing being about 2150° F.

Other examples of powders that may be used are iron and aluminum, with iron in the range of 80% to 90% by weight, and aluminum 10% to 20% by weight. In this case the sintering temperature is on the order of 900° F. or less, and the alloying temperature about 1000° F. or more.

Another example of powders that may be used are copper and titanium powders in a 90% to 10% weight ratio, employing temperatures of 500° F. to 600° F. for sintering and about 1000° F. or more for alloying.

Another example comprises the use of nickel and titanium. In this case the weight of nickel powder would be in the range of 70% to 75%, and the titanium 25% to 30%. In this case the sintering temperature is about 950° F. or less, and the alloying temperature about 1000° F. or more.

The above-listed materials to form alloys are given by way of example and there are others unnecessary to mention because those useful according to the process will be clear from the above.

It may be mentioned that the use of the wetting agent in the slurry is not always required. Thus it is not required when polyethylene oxide, nonionic cellulose ether or polyvinyl pyrrolidone are used as the long-chain, high-molecular-weight organic compound to form the slurry. Also, while in the example the coatings 29 and 31 are applied to strip 1 by roller coating, they could be applied by passing the strip up through a tank, by brushing or by other suitable means for applying a uniform coating on the carrier strip.

It will be understood that although the principles of the invention have been described in reference to three-component and two-component alloys, these principles would be applicable to an alloy consisting of any other number of components, provided the particulate forms of some of the components can be green-bonded and remain nonbrittle at a temperature lower than the temperature required for homogenizing all of them to form the desired alloy which may be brittle.

In view of the above, it will be seen that the several objects of the invention are achieved and other advantageous results attained.

As various changes could be made in the above methods, apparatus and products without departing from the scope of the invention, it is intended that all matter contained in the above description or shown in the accompanying drawings shall be interpreted as illustrative and not in a limiting sense.

What is claimed is:

1. A free substantially nonporous brittle metallic foil of thickness in the range of 0.001 to 0.008 inch, the metal of the foil consisting of a homogeneous alloy sinter without directional grain, the components of said alloy sinter being selected from the following groups, consisting respectively by weight of approximately

- (1) silicon 4.5%, boron 3.5%, nickel 92.0%;
- (2) nickel 71.0%, silicon 10%, chromium 19%;
- (3) iron in the range of 80-90%, aluminum in the range of 10-20%;
- (4) copper 90%, titanium 10%;
- (5) nickel in the range of 70-75%, titanium in the range of 30-25%.

## References Cited

## UNITED STATES PATENTS

- |           |         |             |          |
|-----------|---------|-------------|----------|
| 2,694,790 | 11/1954 | Studders    | 29—182 X |
| 2,900,254 | 8/1959  | Raiklen     | 75—214   |
| 3,144,330 | 8/1964  | Storchchein | 75—226   |
| 3,202,951 | 8/1965  | Krinsky     | 75—138 X |
| 3,203,794 | 8/1965  | Jaffee      | 75—175.5 |
| 3,258,318 | 6/1966  | Grubl       | 29—183   |
| 3,323,879 | 6/1967  | Karstetter  | 29—182   |
| 3,328,166 | 6/1967  | Ayers       | 75—214   |
| 3,335,000 | 8/1967  | Bliss       | 75—208 X |
| 3,387,970 | 6/1968  | Wainer      | 29—183 X |

## FOREIGN PATENTS

- 1,004,457 3/1954 Germany.

## OTHER REFERENCES

- 5 "The Compaction of Metal Powders by Rolling, I.  
The Properties of Strip Rolled from Copper Powders."  
Evans et al., Powder Metallurgy, 1959, No. 3, pp. 1-2.

- 10 BENJAMIN R. PADGETT, Primary Examiner  
A. J. STEINER, Assistant Examiner

U.S. CL. X.R.